

## UNITED STATES PATENT OFFICE

2,431,947

FORMATION OF A STRONG BOND BETWEEN  
A FERROUS METAL SURFACE AND AN  
ELECTRODEPOSIT OF SILVERWilliam M. Martz, Indianapolis, Ind., assignor to  
General Motors Corporation, Detroit, Mich., a  
corporation of DelawareNo Drawing. Application March 6, 1943,  
Serial No. 478,294

2 Claims. (Cl. 204—34)

1

This invention relates to a process of forming a high strength bond between an iron or steel surface and an electrodeposit of silver.

In the production of a silver plated steel surface (such as, for example, steel-backed silver plated bearings) it has been the practice to first electrodeposit a plating of a metal such as copper or nickel onto the steel and then electrodeposit the silver onto the copper or nickel. This has been essential in order to form a strong, adherent plating of silver. I have now found it possible to form a high strength bond directly between electrodeposited silver and steel when the steel surface is given a preliminary treatment, so that the intermediate layer of nickel or copper may be dispensed with.

Broadly stated the invention includes the anodic treatment of the iron or steel surface with a phosphoric acid solution, and the subsequent plating of the silver directly to the treated steel surface. Wetting agents of various kinds compatible with the phosphoric acid solution may be used with beneficial effect. Best results are obtained when the parts are given a cyanide dip prior to silver plating and when the silver plated parts are annealed.

The phosphoric acid may be employed in various proportions. It is preferred that equal volumes of phosphoric acid ( $H_3PO_4$ ) and water be used and that the treatment be carried out at room temperature. However wide variation in the proportions of phosphoric acid and water is permissible and the treatment may be carried out at from room temperature or below up to  $150^{\circ} F.$  or higher.

The cathodes preferably are of stainless steel and should present sufficient surface area so as to permit the use of high anode current densities. The container may be of glass or rubber lined material and should not expose any metal portions to the solution.

The current densities at the anode may vary considerably, current densities on the order of 5 to 150 amperes per square foot or higher being suitable. The higher current densities result in more rapid "cleaning" and in a brighter finish. The time of the anodic treatment is on the order of from 30 to 600 seconds depending on the type of steel being cleaned.

Direct current in the order of 6 or 12 volts is suitable.

After the steel parts are thus treated they are thoroughly washed as by the use of warm running water and thereafter the silver is electrodeposited directly onto the steel. To secure best

2

results the parts are given a cyanide dip before being silver plated. The cyanide solution may be one containing 100 grams of potassium or sodium cyanide per liter of water, although considerable variation in the concentration of cyanide may be employed. The work may be immersed or dipped in the cyanide solution for 10 to 20 seconds.

The steel parts are then given a "strike" or "flash" of silver and thereafter silver plated for the time necessary to give the desired thickness of silver plate. A suitable procedure for forming the "strike" of silver is to provide a silver plating bath composed of 1.5-2.5 grams per liter of  $AgCN$ , and 150 grams per liter of  $KCN$  (free). The temperature of the bath is maintained on the order of  $75-90^{\circ} F.$  The work is "struck" in the bath for a period of 10 to 30 seconds using a current density of 15 to 50 amperes per square foot. The electrical contact must be made prior to immersion in the solution for best results. The parts are removed and thereafter plated with silver in a silver plating bath which preferably contains 130 to 150 grams per liter of  $AgCN$ , 160 to 180 grams per liter of  $KCN$  and 10 to 20 grams per liter of  $KOH$ . The bath may also contain any of the known silver "brighteners" such as, carbon disulfide, ammonium thiosulfate, potassium thiosulfate, etc., if so desired. The bath is operated at a temperature of 100 to  $125^{\circ} F.$  The electrical contact should be made prior to the immersion of the piece in the solution. For best results suitable agitation is provided and the current density permissible depends to a large extent upon this factor.

For best results the silver plated parts are annealed in a neutral or reducing atmosphere at a temperature on the order of  $400$  to  $1200^{\circ} F.$  for about  $\frac{1}{2}$  to 2 hours. The annealing may be carried out in an air atmosphere if the temperature of the work is held below  $900^{\circ} F.$  but a neutral or reducing atmosphere is preferable. The work should be allowed to cool slowly from the annealing temperature.

Before the steel surface is given the anodic treatment in the phosphoric acid solution it is desirable that the surfaces be cleaned as by means of an alkaline cleaning solution. A suitable solution of this sort is composed as follows:

|                   | Per cent                  |
|-------------------|---------------------------|
| $Na_3PO_4$ -----  | 12                        |
| $Na_2SiO_3$ ----- | 38                        |
| $Na_2CO_3$ -----  | 6                         |
| 55 $NaOH$ -----   | 44                        |
|                   | 12 oz. per gal. of $H_2O$ |

The temperature of the alkaline cleaning bath should be 180° to 200° F. during operation. Current densities on the order of 75 to 150 amperes per square foot are satisfactory. The work may be either anode or cathode, preferably anodic. After the alkaline cleaning operation the parts are rinsed thoroughly in warm running water.

To secure best results all of the plating and cleaning solutions must be kept well filtered and free from contaminations, especially oil or metallic particles from the anode or elsewhere.

I claim:

1. A process of producing a strongly bonded electrodeposit of silver directly onto a steel surface which includes, electrolytically cleaning the said surface in an alkaline solution, washing said cleaned steel surface, anodically treating said washed steel surface in a solution composed of approximately equal volumes of phosphoric acid and water for from 30 to 600 seconds, the acid solution being operated at a temperature from about room temperature up to 150° F. and at an anode current density of 5 to 150 amperes per square foot, rinsing said anodic treated surface, then dipping said treated surface in an aqueous cyanide solution composed of approximately 100 grams per liter of an alkali metal cyanide of the class consisting of sodium cyanide and potassium cyanide for about 10 to 20 seconds, striking a silver plate onto said surface in a bath composed of 1.5-2.5 g./liter, silver cyanide, and 150 g./liter potassium cyanide (free), the bath being maintained at a temperature of 75-90° F., a current density of 15-50 amperes per square foot being employed and the time being from 10 to 30 seconds, then electrodepositing a silver plating of desired thickness in a silver plating bath maintained at 100-125° F. and containing 130 to 150 g./liter of silver cyanide, 160 to 180 g./liter of potassium cyanide (free) and 10 to 20 g./liter of potassium hydroxide, and thereafter annealing the silver plated steel surface at a temperature of 400 to 1200° F. for 30 to 120 minutes in a non-oxidizing atmosphere.

2. A process of producing a strongly bonded electrodeposit of silver directly onto a steel surface which includes, electrolytically cleaning the said surface in an alkaline solution, washing said cleaned steel surface, anodically treating said

washed steel surface in a solution composed of approximately equal volumes of phosphoric acid ( $H_3PO_4$ ) and water for from approximately 30 to 600 seconds, the acid solution being operated at a temperature from about room temperature up to 150° F. and at an anode current density of from 5 to 150 amperes per square foot, rinsing said anodically treated surface, then cyanide dipping said treated surface in an aqueous solution of an alkali metal cyanide of the class consisting of sodium cyanide and potassium cyanide for about 10 to 20 seconds, then striking a silver plate onto said surface in a silver cyanide electroplating strike solution, then electrodepositing a silver plate of desired thickness in a silver cyanide plating bath, and thereafter annealing said silver plated steel surface at a temperature within the range of approximately 400° to 1200° F. for a time within the approximate range of 30 to 120 minutes in a non-oxidizing atmosphere.

WILLIAM M. MARTZ.

#### REFERENCES CITED

The following references are of record in the file of this patent:

#### UNITED STATES PATENTS

| Number       | Name     | Date          |
|--------------|----------|---------------|
| 2,104,269    | Oplinger | Jan. 4, 1938  |
| 30 1,916,503 | Wilson   | July 4, 1933  |
| 2,197,653    | Wilson   | Apr. 16, 1940 |
| 1,658,222    | Burns    | Feb. 27, 1928 |
| 2,277,664    | Hull     | Mar. 31, 1942 |
| 35 1,995,766 | Chester  | Mar. 26, 1935 |
| 1,949,713    | Gravell  | Mar. 6, 1934  |
| 1,909,149    | Hitner   | May 16, 1933  |

#### OTHER REFERENCES

Transactions of the Electrochemical Society, 40 vol. 74 (1938), pages 284 and 287-304.

Transactions of the Electrochemical Society, vol. 82 (1943), page 109 (in the discussion of the paper "The Adherence of Thick Silver Plate on Steel," by H. L. Crosby and L. I. Gilbertson, presented at the 82nd General Meeting in Detroit, Michigan, Oct. 8, 1942).

American Electro-plater's Society Monthly Review, vol. 29, (1942), an article by H. Strow on "Metal Cleaning in Wartime," page 996.